

## UNITED STATES PATENT OFFICE

2,225,843

FUR TREATING COMPOSITION AND  
PROCESSWilliam Page, Cranford, and Morris Lefkowitz,  
Irvington, N. J.No Drawing. Application February 10, 1940,  
Serial No. 318,324

7 Claims. (Cl. 8—112)

The present invention is concerned with the production of fur which may be readily processed into felt of improved quality. The invention more particularly is concerned with an improved so-called "carrotting process" by which rabbit, hare, beaver, and similar types of fur are treated, utilizing as a carrotting solution an aqueous mixture comprising a zinc salt, an oxidizing agent, and a hydrolyzing agent. In accordance with the present process, a carrotted fur is produced which may be readily processed into a smooth, strong, tight felt which will exhibit substantially improved wearing qualities. Our process is particularly desirable in that the resulting product is of a higher quality than has heretofore been secured and that this product is secured in an economical and efficient process which is entirely innocuous with respect to the health of the operating personnel.

It is well known in the art to process animal fur, particularly rabbit, hare, beaver, and similar types of fur, by a carrotting process which generally comprises treating the fur with an aqueous solution of mercuric nitrate and nitric acid. This solution is usually applied to the fur while still on the pelt although it may be applied after removal of the fur from the pelt. The fur is then dried at temperatures ranging from atmospheric to temperatures as high as 250° F. or higher, depending upon the nature of the fur and the type and quality of final treated product desired. The drying conditions vary considerably, depending to a large extent upon the particular fur being processed, the carrotting solution employed, as well as upon general atmospheric and other related conditions. However, due to the fact that mercury and mercury salts are toxic in nature and may adversely affect the health of the operating personnel in contact with felting processes and related arts, it has been suggested that various non-mercuric carrotting solutions be substituted for the mercuric carrotting solutions. In general, these mercury-free solutions comprise an oxidation agent, as for example chloric acid, bromic acid, iodic acid, permanganic acid, hydrogen peroxide, and the like, and a hydrolyzing agent, such as sulfuric acid, acids of phosphorus, or equivalent acids with function to duplicate the oxidation and hydrolyzing effects secured by the nitric acid present in the mercuric nitrate solution.

The hydrolyzing agents in general are characterized by having a high ionization value and by being relatively non-volatile at drying temperatures. Desirable hydrolyzing agents, fur-

thermore, are relatively stable so that side reactions resulting in the consumption of the agent do not occur during the processing. Particular non-mercurous carrotting solutions which have been suggested are, for example, a solution comprising an oxidation agent such as permanganic acid and a hydrolyzing agent which is preferably sulfuric acid or a carrotting solution in which the oxidizing agent is a peroxide, as for example, hydrogen peroxide. These solutions, in general, have not been commercially successful due in part to the fact that they have "slow starting" and "slow sizing" characteristics. It is also known that although certain desired results may be secured in the carrotting process, provided the treating reagents are sufficiently strong and concentrated. Other deleterious factors are encountered in that the life of the fiber is adversely affected, particularly with respect to its wearing ability and with respect to its ability to absorb color. Furthermore, when utilizing sulphuric acid as the hydrolyzing agent, increasing the concentrations of the same will tend to cause formation of tarry matter on the surface of the fiber giving it a burnt appearance and rendering it unsuitable for use. In order to overcome the disadvantages of this type of carrotting solution, numerous suggestions have been made for incorporating various inhibiting and catalytic agents into respective non-mercuric solutions which have not produced material benefits, particularly with respect to duplicating the efficiency of the mercuric nitrate solution and the uniform quality of the resulting product.

We have now discovered a non-toxic carrotting solution which may be efficiently employed for the production of a carrotted fur of exceptionally high uniform quality. The carrotted fur produced by our process is extremely stable and may be stored for long periods of time without any substantial deterioration of the fiber occurring. Our carrotted fur may be readily felted with an exceptionally low loss in weight during the felting operation. Furthermore, the felted product produced from our fur is smoothly and tightly interlaced, resulting in the production of a fabric having exceptionally fine, natural lustre and resiliency of the fibers, which in turn contributes to the appearance and wearing quality of the felt. Our felt is also characterized in that it has the ability to absorb and indefinitely retain without fading all dye shades without objectionable overcast or other mottled effects or background.

The carrotting solution of our invention comprises a zinc salt, an oxidizing agent, and a hy-

droyzing agent. Although the zinc salt may comprise the chloride or the nitrate, the preferred zinc salt is the sulfate. The oxidizing agent may comprise any known satisfactory oxidizing agent used in carroting processes, as for example, iodic acid, permanganic acid, hydrogen peroxide, and the like. However, in general, we prefer to employ hydrogen peroxide in combination with the zinc sulfate. The hydrolyzing agent likewise may comprise any satisfactory material which is generally characterized by having a high ionization value and which is relatively non-volatile at the temperatures of drying, as for example, a sulphuric acid, hydrochloric acid, nitric acid, or an acid of phosphorus. In general, however, we have found that particularly desirable results are secured, provided zinc sulfate, hydrogen peroxide, and sulphuric acid be used in conjunction with one another.

The concentration of the particular constituents in our carroting composition may vary considerably depending upon reagents employed. For example when utilizing a preferred composition it is desirable that the concentration of the zinc sulphate be in the range from about 2 to 10% by weight, particularly in the range from about 5 to 7%, that the weight concentration of the hydrogen peroxide based on a hundred volume solution, be about equivalent to or several per cent higher than the weight concentration of the zinc sulphate; and that the weight concentration of the sulfuric acid be about 40% to 60% greater than the concentration of the zinc sulphate, based upon 66° Baumé acid or equivalent. For example, a very satisfactory treating composition consists of an aqueous solution of about 6% by weight of zinc sulphate, about 8% by weight of 100 volume hydrogen peroxide, and about 9% by weight of 66° Baumé sulfuric or its equivalent.

The properties of our solution may be somewhat varied and controlled by the addition thereto of various inhibiting and catalyzing agents. In this regard we have further discovered that the effectiveness and desirability of our solution is considerably enhanced provided a low ionizable organic acid and for example acetic acid and the like be employed in conjunction therewith, and that its value is further enhanced provided a ketone, particularly acetone, is also employed. We have also discovered that the "waste", a loss of weight in felting, is materially reduced provided tannic acid be em-

centrations of the same be from two to three times the weight concentration of the zinc sulphate. The preferred tannic acid concentration is from about 6 to 8% weight per cent. A particular desirable solution consists of from about 5 to 8% by weight zinc sulphate, 5 to 7% tannic acid, 12 to 25% of 28% acetic acid, 5 to 10% of 66° Baumé sulphuric acid and from about 4 to 8% of 100 volume hydrogen peroxide.

In order to further illustrate the invention the following examples are given which should not be construed as limiting the same in any manner whatsoever:

#### Example

A number of carroting and felting operations were conducted utilizing various commercial carroting solutions and carroting solutions within the scope of the present invention. The compositions of the preferred solutions are as follows:

#### Preferred carroting solution—A

|                                        | Weight per cent |
|----------------------------------------|-----------------|
| Zinc sulphate                          | 6               |
| Sulphuric acid, 66° Baumé              | 25              |
| Acetic acid, 28%                       | 16              |
| Hydrogen peroxide, 100 volume solution | 6               |

#### Preferred carroting solution—B

|                                        | Weight per cent |
|----------------------------------------|-----------------|
| Zinc sulphate                          | 5               |
| Sulphuric acid, 66° Baumé              | 9               |
| Acetic acid, 28%                       | 16              |
| Hydrogen peroxide, 100 volume solution | 6               |

#### Preferred carroting solution—C

|                                        | Weight per cent |
|----------------------------------------|-----------------|
| Zinc sulphate                          | 5               |
| Sulphuric acid, 66° Baumé              | 9               |
| Acetone                                | 16              |
| Hydrogen peroxide, 100 volume solution | 8               |

#### Preferred carroting solution—D

|                                        | Weight per cent |
|----------------------------------------|-----------------|
| Zinc chloride                          | 5               |
| Acetic acid, 28%                       | 10              |
| Hydrogen peroxide, 100 volume solution | 6               |

#### Preferred carroting solution—E

|                                        | Weight per cent |
|----------------------------------------|-----------------|
| Zinc sulphate                          | 5               |
| Tannic acid                            | 7               |
| Acetic acid, 28%                       | 15              |
| Sulphuric acid, 66° Baumé              | 7               |
| Hydrogen peroxide, 100 volume solution | 4               |

The results secured when employing the respective solutions are as follows:

| Carroting composition employed    | Appearance of fur after treating, drying and cutting | Percent loss of weight after felting | Felting process shrinking characteristics |                       |                        | Comments   |
|-----------------------------------|------------------------------------------------------|--------------------------------------|-------------------------------------------|-----------------------|------------------------|------------|
|                                   |                                                      |                                      | Starting* (rounds)                        | Machine A** (minutes) | Machine B*** (minutes) |            |
| Commercial mercuric nitrate carro | Good yield, glossy, fibers cling                     | 11                                   | 4                                         | 8                     | 18                     | Very good. |
| Commercial nonmercuric carro, #1  | Poor yield, dull, harsh appearance                   | 28                                   | 3½                                        | 10                    | 22                     | Fair.      |
| Commercial nonmercuric carro, #2  | Fair yield, slightly dull appearance                 | 23                                   | 4½                                        | 12                    | 33                     | Do.        |
| Commercial nonmercuric carro, #3  | Fair yield, fur darkened, some gloss                 | 27                                   | 6½                                        | 18                    | 50                     | Poor.      |
| Commercial nonmercuric carro, #4  | Poor yield, some gloss, pungent (odor)               | 24                                   | 5½                                        | 10                    | 20                     | Do.        |
| Preferred carroting solution (A)  | Good yield, harsh feel                               | 15                                   | 5½                                        | 10                    | 20                     | Good.      |
| Preferred carroting solution (B)  | Good yield, glossy, fibers adhesive                  | 17                                   | 5½                                        | 11                    | 21                     | Very good. |
| Preferred carroting solution (C)  | Good yield, some gloss, harsh feel                   | 20                                   | 5½                                        | 12                    | 26                     | Good.      |
| Preferred carroting solution (D)  | Good yield, some gloss, good appearance              | 21                                   | 6                                         | 12                    | 24                     | Fair.      |
| Preferred carroting solution (E)  | Good yield, glossy, fibers adhesive                  | 3                                    | 5½                                        | 10                    | 20                     | Very good. |

\*Number of times through machine for initial shrinking.

\*\*Time required for shrinking to intermediate predetermined fixed size.

\*\*\*Time required for shrinking to final predetermined fixed size.

ployed in conjunction with our solution. When employing acetic acid or acetone or equivalent reagents it is preferred that the weight con-

centrations of the same be from two to three times the weight concentration of the zinc sulphate. The preferred tannic acid concentration is from about 6 to 8% weight per cent. A particular desirable solution consists of from about 5 to 8% by weight zinc sulphate, 5 to 7% tannic acid, 12 to 25% of 28% acetic acid, 5 to 10% of 66° Baumé sulphuric acid and from about 4 to 8% of 100 volume hydrogen peroxide.

From the above data it is apparent that the carroting solutions of the present invention possess distinct advantages and result in an im-

75

proved product. The felted material furthermore is apparently impregnated in a manner with zinc which materially facilitates the shaping and sizing operations and results in the production of a product of a fine texture and lustre having improved properties with respect to its ability to retain its shape and wear for longer time periods under extremely adverse conditions.

The process of the present invention is not to be limited by any theory or mode of operation but only in and by the following claims by which it is desired to claim all novelty insofar as the prior art permits.

We claim:

- 15 1. A composition for carroting fur comprising zinc sulphate, acetic acid, a peroxidizing agent and an hydrolyzing agent.
- 20 2. A composition as defined by claim 1 in which the concentration of the zinc sulphate is in the range from about 5% to 8% and the concentration of acetic acid is in the range from about 12% to 25%.
- 25 3. A process for the production of fur which may be readily felted comprising treating fur

with a carroting solution comprising zinc sulphate, acetic acid, a peroxidizing agent and an hydrolyzing agent.

4. A process as defined by claim 3 in which the hydrolyzing agent comprises sulfuric acid. 5

5. A composition for carroting fur comprising zinc sulphate, acetic acid, tannic acid, a peroxidizing agent and an hydrolyzing agent.

6. A composition for carroting fur comprising 5% to 8% by weight of zinc sulphate, 5% to 7% 10 of tannic acid, 12% to 25% by weight of 28% acetic acid, 5% to 10% of 60° Baumé sulfuric acid, and from about 4% to 8% of 100 volume hydrogen peroxide.

7. A process for the production of fur which 15 may be readily felted comprising treating fur with a carroting solution comprising 5% to 8% by weight of zinc sulphate, 5% to 7% by weight of tannic acid, 12% to 25% by weight of 28% acetic acid, 5% to 10% of 66° Baumé sulfuric acid, 20 and from about 4% to 8% of 100 volume hydrogen peroxide.

WILLIAM PAGE.  
MORRIS LEFKOWITZ.